

D. DE ROS.

PRODUCTION OF TIN OXID AND ZINC OXID.  
APPLICATION FILED OCT. 30, 1919.

1,372,407.

Patented Mar. 22, 1921.

2 SHEETS—SHEET 1.



Inventor  
Dudley de Ros.  
By Henry Orth Atty

1,372,407.

D. DE ROS.  
PRODUCTION OF TIN OXID AND ZINC OXID.  
APPLICATION FILED OCT 30, 1919.

Patented Mar. 22, 1921.

2 SHEETS—SHEET 2.

FIG. 3.



FIG. 4.



Inventor  
Dudley de Ros,  
By Haunwirth Atty

# UNITED STATES PATENT OFFICE.

DUDLEY DE ROS, OF GREENHITHE, ENGLAND.

## PRODUCTION OF TIN OXID AND ZINC OXID.

1,372,407.

Specification of Letters Patent. Patented Mar. 22, 1921.

Application filed October 30, 1919. Serial No. 334,423.

To all whom it may concern:

Be it known that I, DUDLEY DE ROS, a subject of the King of Great Britain, residing at Black Duck Wharf, Greenhithe, in the 5 county of Kent, England, have invented certain new and useful Improvements in the Production of Tin Oxid and Zinc Oxid, of which the following is a specification.

This invention comprises improvements 10 in and relating to the production of tin oxid and zinc oxid, and relates to processes in which tin or zinc, or a material containing either of these metals, is heated or ignited by means of, for example, an oil fuel burner, 15 and upon the attainment of a sufficiently high temperature in the mass, air or oxygen or oxidizing gas is blown into or applied to the molten mass with the result that exothermic action is set up and an emission of 20 tin oxid or zinc oxid, as the case may be, takes place.

Important objects of this invention are to effect a more perfect and economical oxidation of the metal, to reduce the working expenses, to recover the metal values more 25 exhaustively and to lengthen the life of the plant and render it less liable to injury by the intensive heating and working to which it is subjected.

More specifically the invention has for its 30 object to utilize a combination or primary and secondary or high pressure and low pressure blasts in performing the exothermic reaction, the primary blast being applied to the molten mass through a submerged nozzle and the secondary blast being introduced above the surface of the mass. The function of the high pressure blast is to set up and maintain the exothermic reaction and the low pressure blast, while effecting 35 an economy in power owing to its use necessitating less call upon the high pressure blast, exercises important functions in converting or oxidizing scull formation and 40 in preventing overheating of the furnace lining and parts.

The reason why tin oxid could not hitherto be economically manufactured by blowing cold air through metal was on account 45 of the heavy scull formation and on account of the high temperature generated, which together with the violent ebullition of the metal bath rapidly destroyed the furnace lining. These disadvantages are, according 50 to the present improvements, obviated by using a small volume of high pressure air

which by reason of an exothermic action set up in the body of the metallic bath not only produces a certain amount of oxid but maintains the bath at such a high temperature 60 that upon a low pressure blast being introduced in the region of but above the surface of the bath, the scull (mainly consisting of stannous oxid and stannous stannate— $Sn_2O_3$ ) is oxidized to stannic oxid and large 65 volumes of additional stannic oxid are given off from the boiling or partly boiling bath. Nevertheless, the low pressure blast performs its advantageous function of keeping the heat within such limits as will prevent 70 overheating.

A further specific object of the invention is to adapt a converter type of furnace for the production of the oxid in the manner aforesaid, the furnace or chamber being 75 capable of tilting or rocking so as to cause the molten contents to submerge the primary or high pressure blast nozzle while leaving the secondary nozzle free to deliver 80 a blast above the surface of the molten mass. Such an apparatus lends itself well to the performance of subsidiary operations, as will be hereinafter explained.

Yet another object is to provide a furnace 85 of this kind with a blast box and clearing rod device for the maintenance of full nozzle aperture, by clearing away any scull collecting over and obstructing the said aperture.

In order that the invention may be readily understood, suitable embodiments of the same are given by way of example in the accompanying drawings in which:—

Figure 1 is a sectional elevation of one construction of apparatus according to this invention.

Fig. 2 is a similar view of another construction and

Fig. 3 is a vertical section on the line III—III of Fig. 2.

Fig. 4 is a longitudinal section of another modification.

In the construction of apparatus for carrying out these improvements, as shown in Fig. 1, there may be an elongated cylindrical or other suitably shaped chamber  $a$  mounted on trunnions  $b$  arranged transversely of the longitudinal axis and about half-way along the same. The ends  $a'$  of the chamber  $a$  may be coned or otherwise 105 suitably reduced and one end may be plugged at  $a^2$ , the plug  $a^2$  being fitted with

- a twyer or duct *e* for the introduction of the high pressure blast from a box *e'* fitted with a gland or stuffing box *e<sup>2</sup>* and push rod *e<sup>3</sup>*. The supply connection for the box *e'* is indicated by dotted circles at *e<sup>5</sup>*. The opposite end of the furnace *a* which is unplugged is left open as at *a<sup>3</sup>*, and serves for the introduction of the tin or the like and the flame of an oil flame burner *c*, where such as used, 5 and, in any case, for the introduction of the low pressure blast or current *d*. In the roof or top of the chamber *a* is an opening which may be surrounded by a short uptake *f*, and this serves for drawing off the tin or zinc 10 15 oxid, through a cowl and pipe *f'*. A vertical branch *f<sup>2</sup>* of the pipe may be fitted with a damper and be adapted for drawing off smoke, gases and fumes at starting up of the furnace. The chamber *a* is suitably 20 lined with refractory material in accordance with the usual practice.

At the commencement of an operation, the charge chamber *a* is heated as a preliminary step, to a temperature of, say, about 900° C., 25 30 35 40 45 50 55 60 65 70 75 80 85 90 95 100 105 110 115 120 125 130

in the case of tin. For this heating, the oil flame burner *c* may be employed such burner being supported so that its orifice is right opposite the open end *a<sup>3</sup>* of the chamber *a* when the latter is in the horizontal position which it assumes at the commencement of a run. This preliminary heating may be carried out by a suitable oil burner in the course of about half an hour. When the desired temperature is reached, the chamber *a* is tilted, as shown in chain lines, so as to raise the open end *a<sup>3</sup>* and depress the plugged end *a<sup>2</sup>*. This tilting carries the open end *a<sup>3</sup>* opposite the low pressure blast nozzle *d*, while the high pressure blast nozzle *e* is appreciably submerged by the molten bath. The high pressure blast at *e* is turned on just prior to the tilting but not necessarily the low pressure blast at *d*, and owing to the well known exothermic reaction, the temperature rapidly rises to, say, 1500 to 1700 degrees centigrade, oxid being formed and drawn off. This temperature being reached, the low pressure blast is turned on at *d*, being delivered above the surface of the molten bath, and while keeping down the temperature and preventing it from becoming excessive, this air or oxygen in turn becomes heated and forms additional oxid from the metal in the furnace and converts the scull into stannic oxid, as will be readily understood. The level of the bath is maintained constant by the introduction, from time to time, of fresh quantities of material, and these are pushed down when necessary into the molten contents. The metal is conveniently introduced through the open end *a<sup>3</sup>*. There should preferably be a predetermined relation between the volume of high pressure air and the quantity of metal to be treated in a given time, and this being main-

tained for the attainment of a suitable temperature, the low pressure air may be regulated to suit the instant conditions in the interior of the chamber.

If scull should form at any time and tend 70 to choke the duct or nozzle *e*, the push rod *e<sup>3</sup>* may be operated to clear the duct of the obstruction.

According to a modification, and as shown in Figs. 2 and 3, the elongated chamber *a'* 75 is formed deepest with a curved depression *a<sup>5</sup>* at the middle. The exterior has a transversely rounded bottom *a<sup>6</sup>*, the chamber *a'* being suitably supported upon wheels or rollers *g'* on two or more longitudinally arranged and parallel shafts *g* which form a sort of cradle support for the chamber *a'* and permit it to be rocked from one side to the other as hereinafter explained. The rounded bottom may be fitted with bands or 85 tracks *t* for the wheels *g'* to bear upon. The side or sides *a<sup>7</sup>* *a<sup>7</sup>* of the chamber *a'* is or are perforated and plugged, the plug or plugs *h* receiving high pressure blast fittings *e<sup>4</sup>* as in the previously described construction. These blast nozzles *e<sup>4</sup>* come opposite the greatest depth of the depression *a<sup>5</sup>* and are at a suitable distance above the bottom. One end of the chamber has an opening for the introduction of the burner *c* and the 95 other end of the chamber has an opening for the introduction of the low pressure blast at *d'*. The burner *c* and pipe or nozzle *d'* may be connected with their source of supply in any suitable manner which will allow them to move with the furnace when the latter is rocked. The uptake opening or openings *f<sup>8</sup>* is or are in the top *a<sup>8</sup>* of the chamber as before, but the burner *c* is situated at the end remote from the uptake. It is preferred to 100 arrange the burner *c* near the top and to support a sloping deflector or tile *a<sup>9</sup>* beneath it, the bottom edge of the tile lying beneath an arch or baffle *a<sup>10</sup>*. By this construction and arrangement it is possible to feed in ingots 105 beneath the tile as indicated by dotted lines at *a<sup>11</sup>*. The deflected flame, gases and air form, as it were, a sort of screen in front of the opening through which the ingot enters, somewhat as indicated by the sloping chain 110 lines and prevents exit of tin oxid, flame and vapors. With this construction, the chamber is in the position shown at the start and after the preliminary heating, it is rocked to one side or the other in order that one or other of the high pressure blast nozzles *h* shall be submerged. The low pressure blast *d'* is introduced through its respective end when the proper moment arrives. Now, in order that all the wear and tear shall not 115 take place on one side only of the chamber, the latter may be rocked, after a suitable period of working, so that the nozzle which has been submerged on one side may be raised above the liquid level, and the pre- 120 125 130

viously raised nozzle may be, in turn, submerged. Naturally, it is not only the nozzles which are under consideration but the walls of the chamber, this rocking preceding enabling the wear or deterioration of the lining of the chamber to be equalized on the two sides, as will be readily understood. The nozzles *h* may be fitted with push rods as in the case of the nozzle *e* Fig. 1.

10 In the modification illustrated in Fig. 4, which is similar in most respects to the construction illustrated in Figs. 2 and 3, the separate low pressure blast nozzle is dispensed with and the opening at that end is closed by a plug *i* which may be removable. With this arrangement, the use of the burner nozzle *c* is continued for the introduction of the low pressure blast, a small quantity of oil being permitted to pass into the furnace 15 with such blast from say, the same supply as the burner. The oil ignites as soon as it enters the chamber, and the combustion imparts a certain amount of heat to the air and keeps the temperature up. Therefore, it is possible to adjust the temperature to a 20 nicety, for the proportion of air through the nozzle may be increased to prevent overheating and the proportion of oil may be increased to prevent undue lowering of the 25 temperature. This construction and mode of working are productive of a very white 30 oxid of great purity.

If desired, the secondary blast may have a pressure of, say, .15 to 0.5 pounds per 35 square inch and the primary or high pressure blast may have a pressure of, say, 4 to 5 pounds per square inch. In some cases, however, both blast nozzles may be supplied from the same source and the secondary 40 blast may be adjusted to such proportions as are deemed to be suitable for the instant conditions in the furnace.

In the course of a run, the metal is introduced from time to time, as aforesaid, 45 and is pushed down, if necessary, into the bath. During the run a certain amount of scull is formed consisting of a mixture of stannous oxid, stannous stannate ( $\text{Sn}_2\text{O}_3$ ) and metallic tin. Now owing to the bath 50 being maintained at a high temperature and owing to the introduction of the secondary blast, the low oxids are converted into stannic oxid which is carried away by the fan or other suction means to the condenser.

55 In regard to all that has been said concerning the oxidation of tin, the same may be generally applicable for the oxidation of zinc with little variation as regards practical procedure and with no departure from 60 the principles forming the basis of the present invention.

I claim:—

1. A process for the production of metal oxids by applying an oxidizing blast to a 65 molten mass and utilizing the heat from the

exothermic reaction, which comprises introducing a blast of predetermined proportions through a submerged nozzle, and introducing a secondary blast adjusted to suit instant conditions above the surface of the 70 mass.

2. The process for the production of metal oxids by applying an oxidizing blast to a molten mass and utilizing the heat from the exothermic reaction, which comprises introducing a high pressure blast through a nozzle submerged in the mass, and introducing a low pressure blast above the surface of the 75 mass.

3. The process for production of metal 80 oxids by applying oxidizing blast to the molten mass and utilizing the heat from the exothermic reaction, which comprises starting the reaction by means of an atmospheric burner, continuing the reaction by a submerged blast, and controlling the instant 85 conditions by a blast continued through said burner.

4. A furnace or hearth for the production 90 of metal oxid by the process described, comprising a chamber tiltably mounted on its support and provided with an aperture for the introduction of flame or heat, a primary blast connection on said furnace, said connection being arranged so that it is submersible upon tilting the chamber, and secondary blast means adapted for delivering a secondary blast into the tilted chamber 95 above the surface of the molten contents, substantially as set forth.

5. A furnace or hearth for the production 100 of metal oxid by the process described, comprising a chamber adapted to tilt laterally on its support and provided with an aperture for the introduction of flame or heat, a primary blast connection at each side of said chamber so disposed that one connection or the other is submersible by the tilting of the chamber toward one side or the other, and means adapted for introducing blast into 105 the upper part of said chamber and above the surface of the molten contents, substantially as set forth.

6. A furnace or hearth for the production 110 of metal oxid by the process described, comprising a chamber supported so as to be revolvable about a longitudinal axis and provided with an aperture for the introduction of flame or heat, a blast connection at each side of said chamber so disposed that one 115 connection or the other is submersible by a partial revolution of said chamber, and a secondary blast adapted to deliver blast above the surface of the molten contents through an aperture formed in an end wall 120 about on the said axis, substantially as set forth.

7. A furnace or hearth for the production 125 of metal oxid by the process described, comprising a chamber adapted to tilt from side 130

to side about a longitudinal axis and formed in one end wall with an aperture about on the said axis, an atmospheric burner arranged opposite said aperture, and a blast connection at each side of said chamber so disposed that one connection or the other is submersible by tilting the furnace to one side or the other, the said aperture being adapted to leave a clear opening for the delivery 10 from the burner at any working angle of tilt, substantially as set forth.

8. A furnace or hearth for the production of metal oxide by the process described, comprising a chamber adapted to tilt, a blast nozzle connected with said chamber and so disposed as to be submersible by the tilting of said chamber, a stuffing box associated with said nozzle, a clearing rod 15 slideable in said box, and means adapted for introducing blast in the chamber above the

surface of the molten contents, substantially as set forth.

9. A furnace or hearth for the production of metal oxide by the process described, comprising a chamber adapted to tilt, a blast 25 nozzle connected with said chamber and so disposed as to be submersible by the tilting of said chamber, means for introducing a secondary blast into said chamber above the surface of the molten contents, a deflector 30 arranged in an aperture in a wall of said chamber and dividing said aperture into a feed inlet passage and a flame and gas inlet passage, and a baffle arranged forwardly of said deflector and adapted to coöperate with 35 said deflector to direct a fluid screen across said feed inlet passage, substantially as set forth.

DUDLEY DE ROS.